

## UNITED STATES PATENT OFFICE.

FREDERICK M. BECKET, OF NEW YORK, N. Y., ASSIGNOR TO ELECTRO METALLURGICAL COMPANY, A CORPORATION OF WEST VIRGINIA.

MANUFACTURE OF TUNGSTEN ALLOYS LOW IN TIN AND ARSENIC.

No Drawing.

Application filed December 11, 1926. Serial No. 154,307.

The invention relates to the treatment of tungsten ores for the recovery of their tungsten content.

The common tungsten ores carry the element in the form of tungstates. For example, ferberite may be regarded as an iron tungstate, wolframite as an iron and manganese tungstate, and scheelite as a calcium tungstate. Such ores can be reduced without special difficulty in the electric furnace, and the tungsten present recovered as an alloy. It is the general practice to recover the tungsten as an alloy with iron since the melting point is lowered as the content of iron increases, and the iron is unobjectionable where the tungsten is ultimately to form part of a ferrous alloy. The tungsten ore itself often contains sufficient iron to produce a suitable alloy with the tungsten.

Tungsten ores in general, however, carry other impurities which are objectionable unless separated from the tungsten. Among such impurities are tin and arsenic, and these are practically always present. Since the tungsten content of high-speed steels is usually between 15% and 20%, it will be evident that the ratio of tin to tungsten or of arsenic to tungsten must be very low in the alloy which is incorporated in making such steels.

The invention is a process for the manufacture of alloys low in tin and arsenic from tungsten ores contaminated with these elements or either of them.

I have discovered that if tungsten ores are reduced by an excess of silicon or silicon alloy or if tungsten and silicon are reduced in the same charge, so that the alloy produced has a considerable content of silicon, a part only of the tin present will enter the alloy. The recovery of tin, by which is meant the proportion of the total tin in the charge which enters the alloy recovered, appears to diminish progressively as the silicon content of the alloy increases. The elimination of arsenic occurs in similar fashion. The percentage of silicon which it will be necessary to incorporate into the alloy will depend on the degree of contamination of the ore and on the specifications for tin and arsenic in the ferrotungsten

produced, but in many cases a silicon content between 10% and 35% is advantageous. Somewhat lower percentages of silicon are effective under some conditions. A silicon content in excess of 20% is usually preferred. The presence of the silicon lowers the melting point of the alloy and facilitates tapping.

The furnace charge for producing the ferrotungsten-silicon contains the tungsten ore and silicon (preferably in the form of high-silicon ferro alloy) to reduce the ore and furnish the requisite excess of silicon. The silicon may be replaced, in whole or in part, by quantities of silica and carbon equivalent thereto. The silica in the ore is of course available for reduction to silicon, and low-grade ores can be employed and their silica content utilized for this purpose.

Ferrotungsten-silicon as such is not a suitable material for addition to ferrous alloys such as high-speed steel since its silicon content is too high. In accordance with the preferred embodiment of my invention, the alloy low in tin and arsenic prepared as described above is therefore treated to oxidize the excess of silicon. A metal oxide is preferably used for this oxidation and as a result the metal of the oxide enters the alloy. An oxide of any metal which is not detrimental to the alloy may be used, but an oxidized tungsten compound such as one of the common tungsten minerals is preferably used. A further quantity of tungsten is thereby added to the ferrotungsten.

Where a tungsten ore is used in the second stage of the process it may likewise be one which is contaminated with tin and arsenic. This is because there is an elimination of these elements in the second stage as well as the first, and also because any impurities which enter in the second stage are diluted by the high grade alloy produced in the first stage. Exclusion of tin and arsenic is not as effective in the second stage as in the first, however, and it is desirable to use an ore low in the impurities in question in the second stage. My invention contemplates a two-stage process in which the available ore which is most contaminated with tin and arsenic,

is used in the first stage and ore relatively free from these impurities is used in the second stage.

A specific example of the process will now 10 be described.

Ferrotungsten-silicon was made by reducing a mixture of wolframite and quartzite with carbon in an electric furnace. The materials used during the run were:

|                                  | Pounds. |
|----------------------------------|---------|
| Wolframite                       | 15,612  |
| Quartzite                        | 7,806   |
| Carbon (coke, coal and charcoal) | 7,462   |
| Fluorspar                        | 200     |
|                                  | 31,080  |

The recovery of tungsten as ferrotungsten-silicon was 93.15%. The wolframite and the 20 alloy produced analyzed as follows:

|    | Wolframite | Ferrotungsten-silicon |
|----|------------|-----------------------|
|    | Per cent.  | Per cent.             |
| W  | 53.05      | 56.39                 |
| Fe | 10.34      | 11.47                 |
| Mn | 8.05       | 6.92                  |
| Si | 18.74      |                       |
| As | 1.36       | 0.23                  |
| Sn | 0.17       | 0.022                 |

30 Over 80% of tin and a like proportion of the arsenic were eliminated.

The ferrotungsten-silicon thus produced was used to reduce a mixture of 7000 lbs. of wolframite which had been magnetically 35 treated for elimination of tin, and 6500 lbs. of scheelite. The analyses of the ores and the final alloy are as follows:

|    | Scheelite | Wolframite | Ferrotungsten |
|----|-----------|------------|---------------|
|    | Per cent. | Per cent.  | Per cent.     |
| W  | 56.11     | 56.87      | 80.98         |
| Fe | 1.30      | 11.02      |               |
| Mn | 0.22      | 8.42       | 0.89          |
| Si |           |            | 0.44          |
| Sn | 0.04      | 0.08       | 0.09          |
| As | 0.005     | 0.039      | 0.020         |

The overall recovery of tungsten in the entire process was approximately 90%.

50 The following additional example of the production of ferrotungsten-silicon shows the influence of a higher content of silicon in excluding tin. The ore was a wolframite containing:

|    | Per cent. |
|----|-----------|
| W  | 53.39     |
| Fe | 13.07     |
| Sn | 0.49      |

The furnace charge contained ore, quartzite and carbon. The alloy produced contained:

|    | Per cent. |
|----|-----------|
| W  | 53.2      |
| Fe | 12.5      |
| Si | 27.6      |
| Sn | 0.04      |

60  
65

I claim:

1. Process of making tungsten alloys low in tin and arsenic from ores contaminated with these elements which comprises reducing the ore, alloying silicon with the tungsten 70 as reduced to produce an alloy containing at least 10% of silicon, and then oxidizing the major portion of the silicon content with a metal oxide in which the ratio of the total reducible metals to the total tin and arsenic 75 is higher than in the ore first reduced.

2. Process of making tungsten alloys low in tin and arsenic from ores contaminated with these elements which comprises reducing the ore, alloying silicon with the tungsten 80 as reduced to produce an alloy containing at least 10% of silicon, and then oxidizing the major portion of the silicon content with a tungsten ore in which the ratio of the total reducible metals to the total tin and arsenic 85 is higher than in the ore first reduced.

3. Process of making tungsten alloys low in tin and arsenic from ores contaminated with these elements which comprises reducing the ore, alloying silicon with the tungsten 90 as reduced to produce an alloy containing at least 10% of silicon, and then oxidizing the major portion of the silicon content with a tungsten ore lower in tin and arsenic than that first referred to.

4. Process which comprises smelting a tungsten-containing material contaminated with tin and arsenic, incorporating at least 10% of silicon into the reduction product, and then desiliconizing the reduction product 100 with a metal oxide in which the ratio of total reducible metals to the total tin and arsenic is higher than in the material first smelted.

5. Process which comprises smelting a tungsten-containing material contaminated with tin and arsenic, incorporating at least 10% of silicon into the reduction product, and then desiliconizing the reduction product with a tungsten ore in which the ratio of total reducible metals to the total tin and arsenic 110 is higher than in the material first smelted.

In testimony whereof, I affix my signature.

FREDERICK M. BECKET.